

## UNITED STATES PATENT OFFICE.

HENRY DREYFUS, OF LONDON, ENGLAND.

## MANUFACTURE OF TEXTILE FABRICS.

No Drawing.

Application filed August 13, 1923. Serial No. 657,222.

*To all whom it may concern:*

Be it known that I, HENRY DREYFUS, a citizen of the Swiss Republic, of London, England, have invented certain new and useful Improvements in or Relating to the Manufacture of Textile Fabrics, of which the following is a specification.

This invention relates to the manufacture of fabrics consisting wholly or partly of 10 yarns or threads of cellulose acetate, or other esters of cellulose or ethers of cellulose all of which are hereinafter included in the term organic derivatives of cellulose, and its object is to produce fabrics of this 15 character presenting new or improved crêpe-like effects.

As is well known, permanent crêpe effects 20 on fabrics made with yarns of natural silk, are obtained by employing highly twisted silk yarns in the gummed state in weaving the fabric, and subsequently boiling off wholly or partly the silk gum, which usually constitutes about 20-25 per cent of the 25 weight of the silk fibre, and drying, the crêpe effect being thus obtained. Usually it is only weft yarns which are highly twisted, but in some cases both weft and warp 30 yarns having a high twist are employed. In most cases one employs both right hand 35 twisted yarns and left hand twisted yarns in the fabric in order to obtain a flat lying fabric; for example right hand twisted weft yarns may alternate with left hand twisted weft yarns in the fabric or be woven in other desired relation thereto.

Hitherto it has not been possible to obtain permanent crêpe effects in fabrics with 40 yarns or threads of cellulose acetate or other esters or ethers of cellulose. Trials made with this object have failed. It has been found that the reason for the inapplicability is that the said yarns or threads, especially cellulose acetate yarns or threads owing to their being somewhat ductile, lose 45 part of their elasticity under the effect of the high twist which is put into them for use as crêpe effect threads, and do not regain their elasticity completely, a permanent stretch being in fact imparted to them under the strain of the high twist so that they 50 are not capable of the necessary degree of shrinkage in fabrics when these are dried after wetting or moistening.

It has now been found that this difficulty 55 can be overcome by providing the said yarns or threads (hereinafter referred to as yarns),

with a protective coating of a colloid substance before they receive the high or relatively high twist; it has been found that by this means the elasticity of said yarns can 60 be preserved or substantially preserved under the strain of the high twist, thus counteracting their tendency to acquire a permanent stretch or elongation in the twisting operation. The yarns thus protected, 65 after receiving the necessary high or relatively high twist (hereinafter for brevity included in the term high twist) are employed as weft yarns, or it may be in both warp and weft, in weaving the fabrics, and 70 when the fabrics are subsequently wetted and dried, the said yarns produce a permanent crêpe effect by their shrinkage. The elasticity preserving coating is wholly or 75 partly removed from said yarns in the woven fabric by any suitable bath or liquid, and the operation of removing said coating may with advantage at the same time serve as the crêping wetting.

Trials have shown that a permanent crêpe 80 effect can only be satisfactorily obtained in fabrics with yarns of cellulose acetate or other esters or ethers of cellulose if these yarns are provided with an elasticity preserving coating as referred to before receiving the necessary high twist. This is 85 a surprising fact, as other yarns such as wool and cotton will give permanent crêpe effects without special protection.

In carrying out the invention I employ 90 high twist yarn of cellulose acetate or other ester or ether of cellulose, which yarn, before receiving the high or relatively high twist, has been treated or impregnated 95 with an elasticity preserving coating or dressing of a colloid substance. The said coating or dressing may consist of any suitable colloidal materials or preparations. For example one may treat or impregnate the said yarns or threads 100 with boiled-off liquor or with solutions or preparations containing gums, gelatine, starch, glucose, so called "sizes" or sizing preparations, especially those consisting of or capable of leaving on the yarns a 105 dressing or coating of a plastic or semi-plastic character consisting for example of starch, glucose and oil, or with mixtures of or containing any of the foregoing, or with 110 any other suitable dressings or preparations. I weave fabrics with weft yarns of such coated or dressed highly or relatively

highly twisted yarns and I afterwards remove the coating or dressing wholly or partly from the said yarns by treating the fabric with boiling or hot water or soap 5 solutions or with other suitable baths or other suitable means.

This operation of removing the coating or dressing preferably serves as the wetting treatment of the crêping operation, the 10 fabrics being subsequently dried, usually under stentering or like tension in order to secure the right width of the crêpe effect fabric. It is understood, however, that a separate crêping wetting treatment may be 15 applied to the fabrics after removal of the protective coating or dressing from the yarns provided therewith, and generally that any known or suitable baths or wetting means may be employed for the purpose or 20 any other suitable means may be applied for effecting the crêping shrinkage.

The weft may consist wholly of the highly or relatively highly twisted and coated or dressed yarns of cellulose acetate or other 25 organic derivatives of cellulose, or partly of such yarns and partly of yarns of other material. The warp may consist of yarns of cellulose acetate or other organic derivatives of cellulose, or of yarns of other material or 30 materials, or partly of yarns of cellulose acetate or other organic derivatives of cellulose and partly of yarns of other material or materials. The warp yarns will usually be of relatively low twist or much lower 35 twist than the crêpe effect weft yarns, but in some cases highly twisted or relatively highly twisted warp yarns may be employed. When warp yarns of cellulose acetate or other esters or ethers of cellulose are employed 40 these may likewise be provided with a coating or dressing such as referred to.

The high or relatively highly twisted coated weft yarns of cellulose acetate or other organic derivatives of cellulose may 45 of course be employed throughout the fabric or only at desired parts thereof according to whether the crêpe effect to be obtained with them shall extend generally over the fabric or only appear at parts. The weaving 50 may in fact be generally similar to that practised in making fabrics with permanent crêpe effects, and the crêpe-effect-producing yarns may be of opposite twists as before referred to in order to secure a flat lying 55 fabric.

The degree of twist imparted to the yarns of cellulose acetate or other organic derivatives of cellulose serving to give the crêpe effect may be similar, to what is usual in 60 weft yarns in the manufacture of silk crêpe, crêpe de chine, crêpe marocain or other crêpes by the known methods, but any other suitable high or relatively high twist may be employed.

The crêpe effect may be more or less pro-

nounced or of any desired degree, according to the number of twists given to the yarns and to the degree of shrinkage. Also any desired deniers of yarns may be used, as for instance 30, 45, 50, 60, 100, 150, 200 70 and more. High deniers may in particular be used with preference for fabrics such as crêpe marocain. It is also to be understood that the deniers employed may consist of a single "end" or be built up of two or more "ends" to make the total denier. In the latter case the "ends" may be separately coated or dressed before being twisted together or before receiving the high or relatively high twist. 80

The yarns of cellulose acetate or other organic derivatives of cellulose employed for the purposes of the invention will usually be composed of continuous filaments, though in some cases they may be spun from short length or chappe cellulose acetate fibres. 85

It is to be understood as before indicated that two or more "ends" of cellulose acetate or other organic derivatives of cellulose may be twisted together with a high or relatively high twist for use as crêpe producing weft yarns. 90

In carrying out the invention, according to one example, to make a crêpe fabric of 45 denier for instance, I may take a 45 denier yarn of cellulose acetate, ethyl, methyl, benzyl cellulose or other ester or ether of cellulose and treat or impregnate it with boiled off liquor or other suitable sizing, dressing or preparation of a suitable concentration so as to apply or leave on the yarn the desired amount of coating or solid material, for instance an amount about corresponding to that of the gum on natural silk, for example about 20-25 per cent, or any desired less or greater amount, for instance between 5 and 20 per cent or 25-30 per cent or more, or even as low as between about 1 and 5 per cent. The yarn, dried if required, is given a suitably high twist, for instance a twist of between 44 and 86 turns per inch, or more or less than this, and is woven as weft into a fabric with warp yarns of cellulose acetate or other cellulose ester or cellulose ether or other material, of the same denier as the weft threads, but of an ordinary degree of twist or of lower twist than said weft, for example of about 5 turns per inch. The warp yarn employed may or may not be coated or dressed similarly to the weft. The woven fabric is then boiled or heated with water or in a soap bath or treated with any other suitable bath to remove the coating or dressing from the yarns and is dried under tension, and a fabric is thus obtained presenting the permanent crêpe effect. 110

It is of course understood that the foregoing example is given only by way of illustration and can be varied widely. 125 130

One may of course employ in the fabric 5 yarns consisting respectively of different esters or ethers of cellulose, or yarns or threads consisting respectively of ester and ether of cellulose, for example yarns of cellulose acetate and yarns of another ester of cellulose, or yarns of cellulose acetate and yarns of cellulose ether. Or yarns may be employed which are composed or built up 10 of two or more of any of the said cellulose derivatives.

It is understood that the number of weft 15 yarns employed in carrying out the invention should not be too great relatively to the number of warp yarns, as otherwise the crêping effect obtained after the shrinkage may be prejudiced. For this reason the 20 number of weft yarns per inch counted lengthwise of the fabric should be substantially less than the number of warp yarns per inch counted transversely of the fabric. For instance with a fabric of 180 warp 25 yarns per inch one may use about 40 to 80 weft yarns per inch, it being of course understood that any other suitable numbers than these may be employed.

In some cases the fabrics produced according to the invention may be treated with a swelling agent or agents for the yarns of cellulose acetate or other cellulose esters or ethers, it having been found that such treatment with a swelling agent can accentuate or increase the crêping effect on the highly twisted yarns of organic derivatives of cellulose. For example one may treat the fabric in a bath of dilute acetic acid, or a bath containing a thiocyanate such as thiocyanate of ammonium or thiocyanate of sodium or other alkali thiocyanate; or any other suitable swelling agents may be employed for the purpose, the fabric being afterwards dried preferably under tension. The swelling treatment may be applied after the removal of the coating or dressing from the cellulose acetate yarns, or before such removal, or it may itself serve at the same time as means for removing the coating or dressing.

What I claim and desire to secure by Letters Patent is:—

1. Process for the production of yarns for use in the manufacture of crêpe fabrics, comprising applying an elasticity preserving coating to yarn composed of organic derivative of cellulose, and twisting said coated yarn with a high twist.

2. Process for the production of yarns for use in the manufacture of crêpe fabrics comprising applying an elasticity preserving coating of colloid substance to yarn composed of organic derivative of cellulose, and twisting said sized yarn with a high twist.

3. In a process for the manufacture of crêpe effect fabrics, the employment of high twist weft yarns of organic derivative of

cellulose having an elasticity preserving coating applied to them prior to receiving the high twist.

4. In a process for the manufacture of crêpe effect fabrics, the employment of high twist weft yarns of cellulose acetate having an elasticity preserving coating applied to them prior to receiving the high twist.

5. In a process for the manufacture of crêpe effect fabrics, the employment of high twist weft yarns of cellulose acetate having an elasticity preserving colloid substance applied to them prior to receiving the high twist.

6. In a process for the manufacture of fabric presenting a permanent crêpe effect, weaving a fabric with high twist weft yarns of organic derivative of cellulose having an elasticity preserving coating of colloid substance applied to them prior to receiving the high twist, and subsequently removing the coating at least partially from said yarns in the woven fabric.

7. In a process for the manufacture of fabric presenting a permanent crêpe effect, weaving a fabric comprising high twist weft yarns of organic cellulose derivative having an elasticity preserving coating of colloid substance applied to them prior to receiving the high twist, and subsequently removing the coating at least partially from said yarns in the woven fabric by treatment of the fabric with a liquid capable of dissolving off the coating.

8. In a process for the manufacture of fabric presenting a permanent crêpe effect, weaving a fabric with high twist weft yarns of organic cellulose derivative having an elasticity preserving coating of colloid substance applied to them prior to receiving the high twist, and subsequently removing the coating at least partially from said yarns in the woven fabric by treatment of the fabric with a hot aqueous liquid.

9. In a process for the manufacture of fabric presenting a permanent crêpe effect, weaving a fabric with high twist weft yarns of organic cellulose derivative having an elasticity preserving coating of colloid substance applied to them prior to receiving the high twist, and subjecting the woven fabric to wetting and drying.

10. In a process for the manufacture of fabric presenting a permanent crêpe effect, weaving a fabric with high twist weft yarns of organic derivative of cellulose having an elasticity preserving coating of colloid substance applied to them prior to receiving the high twist, and subsequently removing the coating at least partially from said yarns in the woven fabric by treatment of the fabric with an aqueous liquid, said treatment likewise serving as wetting treatment for the crêping, and drying the fabric.

11. In a process for the manufacture of

1  
fabric presenting a permanent crêpe effect, weaving a fabric with high twist weft yarns of organic derivative of cellulose having an elasticity preserving coating of colloid substance applied to them prior to receiving the high twist, treating the woven fabric with a hot aqueous liquid whereby said coating is at least partially removed from said coated high twist weft yarns said treatment 10 likewise serving as wetting treatment for the crêping, and drying the fabric.

12. In a process for the manufacture of fabric presenting a permanent crêpe effect, weaving a fabric with high twist weft yarns 15 of cellulose acetate having an elasticity preserving coating of colloid substance applied to them prior to receiving the high twist, and subsequently removing the coating at least partially from said yarns in the woven 20 fabric by treatment of the fabric with a liquid capable of dissolving off the coating;

13. In a process for the manufacture of fabric presenting a permanent crêpe effect, weaving a fabric with high twist weft yarns 25 of cellulose acetate having an elasticity preserving coating of colloid substance applied to them prior to receiving the high twist, and subsequently removing the coating at least partially from said high twist cellulose acetate yarns in the woven fabric by 30 treatment with a hot aqueous liquid, and drying the fabric.

14. In a process for the manufacture of fabric presenting a permanent crêpe effect, 35 weaving a fabric with high twist weft yarns of cellulose acetate having an elasticity preserving coating of colloid substance applied to them prior to receiving the high twist, and subjecting the woven fabric to wetting 40 and drying.

15. In a process for the manufacture of fabric presenting a permanent crêpe effect, weaving a fabric with high twist weft yarns of cellulose acetate having an elasticity preserving coating of colloid substance applied to them prior to receiving the high twist, and subsequently removing the coating at 45 least partially from said yarns in the woven fabric by treatment of the fabric with an aqueous liquid, said treatment likewise serving 50 as wetting treatment for the crêping, and drying the fabric.

16. In a process for the manufacture of fabric presenting a permanent crêpe effect, 55 weaving a fabric with high twist weft yarns of cellulose acetate having an elasticity preserving coating of colloid substance applied

to them prior to receiving the high twist, treating the woven fabric with a hot aqueous liquid whereby said coating is at least partially removed from said coated high twist cellulose acetate yarns, said treatment likewise serving as wetting treatment for the crêping, and drying the fabric.

17. In a process for the manufacture of fabric presenting a permanent crêpe effect, weaving a fabric with high twist weft yarns of organic derivative of cellulose having an elasticity preserving coating of colloid substance applied to them prior to receiving the high twist, and treating the fabric with a solution of a chemical swelling agent for 70 said yarns of organic cellulose derivative.

18. In a process for the manufacture of fabric presenting a permanent crêpe effect, 75 weaving a fabric with high twist weft yarns of organic derivative of cellulose having an elasticity preserving coating of colloid substance applied to them prior to receiving the high twist, treating the fabric with a 80 solution of a chemical swelling agent for said yarns of organic cellulose derivative and removing said protective coating at least partially from said yarns.

19. In a process for the manufacture of fabric presenting a permanent crêpe effect, weaving a fabric with high twist weft yarns of organic derivative of cellulose having an elasticity preserving coating of colloid substance applied to them prior to receiving the high twist, treating the fabric with an aqueous solution of a chemical swelling agent for said yarns of organic cellulose derivative, thereby removing the coating at 90 least partially from said yarns and swelling them, and thereafter drying the fabric.

20. As new products applicable for the manufacture of crêpe fabrics, high twist yarns of organic derivative of cellulose, 95 said yarns comprising a coating of colloid substance whereby elasticity of said yarns is preserved under the high twist.

21. As new products, woven fabrics comprising high twist weft yarns of organic derivative of cellulose and presenting a 100 permanent crêpe effect.

22. As new products, woven fabrics comprising high twist weft yarns of cellulose acetate and presenting a permanent crêpe effect.

In testimony whereof I have hereunto subscribed my name.

HENRY DREYFUS.